

July 6, 1937.

F. R. HENSEL ET AL

2,086,329

COPPER ALLOY

Filed May 26, 1936



INVENTORS  
Franz R. Hensel  
BY Earl I. Larsen  
R. H. H.  
ATTORNEY

## UNITED STATES PATENT OFFICE

2,086,329

## COPPER ALLOY

Franz R. Hensel and Earl I. Larsen, Indianapolis,  
Ind., assignors to P. R. Mallory & Co., Inc.,  
Indianapolis, Ind., a corporation of Delaware

Application May 26, 1936, Serial No. 81,820

5 Claims. (Cl. 75—153)

This invention relates to alloys and more particularly to copper alloys of improved characteristics.

An object of the invention is to produce an improved copper base alloy.

Another object is to produce a copper cadmium alloy which can be age-hardened.

Other objects of the invention will be apparent from the following description taken in connection with the appended claims.

The present invention comprises the combination of elements, methods of manufacture, and the product thereof brought out and exemplified in the disclosure hereinafter set forth, the scope 15 of the invention being indicated in the appended claims.

In the drawing:

Figure 1 is a graph having curves illustrating the improvement in the hardness and electrical 20 conductivity of the alloy of the present invention during age-hardening;

Figure 2 is a graph showing the effect of temperature on the hardness of the finished alloy; and

Figure 3 is a graph showing the effects of cold working the alloy.

While a preferred embodiment of the invention is described herein, it is contemplated that considerable variation may be made in the method 30 of procedure and the combination of elements without departing from the spirit of the invention.

Copper-cadmium alloys are frequently used at the present time for resistance welding electrodes, 35 spot welding electrodes, trolley wires, trolley wheels and electrical contactors of various types. These alloys, while having numerous advantages when used at low temperatures, are not entirely satisfactory when used even at moderately high 40 temperatures such as 300 to 350° C. According to the present invention these alloys are improved by the addition of zirconium. The improved alloys can not only be made of greater hardness than prior copper-cadmium alloys but are also 45 capable of retaining their hardness at higher temperatures.

According to the preferred method of carrying out the present invention an alloy is made containing copper, cadmium and zirconium in substantially the following proportions:

|           |            |
|-----------|------------|
| Cadmium   | 0.1% to 2% |
| Zirconium | 0.1% to 5% |
| Copper    | Balance    |

55 It is possible likewise to improve the character-

istics of other copper-cadmium alloys containing small percentages of additional ingredients by the addition of zirconium. Thus copper-cadmium alloys containing small proportions of silver, zinc, calcium, lithium, silicon or beryllium can be improved by the addition of zirconium in substantially the proportions indicated above.

The addition of zirconium to the above alloys renders them susceptible to age-hardening.

The alloy can be made according to standard 10 alloying methods. A preferred method of alloying is to prepare a "hardener alloy" containing 10-30% zirconium and then introduce a predetermined amount of this alloy into a copper-cadmium alloy of the desired composition. 15

After the alloy has been prepared according to standard alloying methods the heat treatment may be carried out as follows: The alloy in the form of a billet or any other form is raised in temperature to above 700° C. and preferably to 20 a temperature in the order of 800° C. to 1000° C. The alloy is then quenched from this high temperature and subsequently aged at a temperature below 700° C. and preferably in the range between 400° C. and 600° C. This heat treatment 25 results in a considerable improvement in hardness of the alloy. For example, an alloy having a Rockwell B hardness of 20 before the quenching and heat treatment may be given a Rockwell B hardness of 60 or greater by the heat treating 30 process. Curve 10 in Figure 1 shows the increase in hardness during the age-hardening step of the heat treating process for an alloy of 1% cadmium, 1% zirconium and the balance copper.

Another remarkable effect of the heat treatment 35 is a marked improvement in electrical conductivity. With some alloy combinations within the percentage range given above a conductivity of 75% of that of pure copper has been obtained. Curve 11 in Figure 1 shows the improvement in 40 conductivity during age-hardening of the same alloy as that whose hardness is represented in curve 10.

This alloy is, therefore, well suited for use at 45 comparatively high temperatures since the hardness and electrical conductivity are maintained for indefinite periods at the aging temperatures indicated. Cold worked and heat treated alloys of the present invention held for two hours at 450° C. retained a Rockwell B hardness of over 50 50. In Figure 2, curve 12 illustrates the maintenance of hardness of a finished alloy at elevated temperatures, the alloy being of the composition mentioned in connection with Figure 1.

In addition to hardening by the heat treat- 55

ment described the above alloys are also susceptible to hardening by cold working. The Rockwell B hardness, in one instance, can be raised from 58 Rockwell B to 80 Rockwell B by 5 giving the material a 40% reduction by cold working. The tensile strength is also increased by cold working. With the above-mentioned alloy containing 1% cadmium and 1% zirconium a tensile strength of 72,000 p. s. i. with 20% 10 elongation has been obtained after 30% cold reduction. Curve 13 in Figure 3 illustrates the improvement in hardness with cold working for the above alloy.

The alloys prepared as indicated above are well 15 suited for the manufacture of castings such as commutator segments and collector rings for dynamo electric machines. In addition, as indicated above, these alloys are suitable for welding electrode tips and welding wheels. They are 20 also useful as current collecting nozzles on automatic arc welding heads.

Another important use of these high strength 25 alloys is in the manufacture of cylinder heads, pistons and other parts of internal combustion engines, such as automobile engines, where high heat conductivity is needed.

While the present invention, as to its objects and advantages, has been described herein as carried out in specific embodiments thereof, it 30 is not desired to be limited thereby but it is intended to cover the invention broadly within the spirit and scope of the appended claims.

What is claimed is:

1. An alloy containing about 0.1 to 2% cadmium, 0.1 to 5% zirconium and the remainder copper.
2. An alloy containing about 0.1 to 2% 5 cadmium, 0.1 to 5% zirconium and the remainder substantially all copper, characterized by a combination of high hardness and high electrical conductivity and further characterized by the ability to maintain its hardness and high conductivity at temperatures in the order of 500° C. 10
3. An age hardened alloy containing about 0.1 to 2% cadmium, 0.1 to 5% zirconium and the remainder substantially all copper, characterized by a combination of high hardness and high 15 electrical conductivity and further characterized by the ability to maintain its hardness and high conductivity at temperatures in the order of 500° C.
4. A welding electrode composed of about 0.1 to 2% cadmium, 0.1 to 5% zirconium and the remainder copper. 20
5. A welding electrode composed of about 0.1 to 2% cadmium, 0.1 to 5% zirconium and the remainder substantially all copper, characterized 25 by a combination of high hardness and high electrical conductivity and further characterized by the ability to maintain its hardness and high conductivity at temperatures in the order of 500° C. 30

FRANZ R. HENSEL.  
EARL I. LARSEN.